

C. E. CARPENTER,  
COMPOSITE LEATHER BELT,  
APPLICATION FILED FEB. 5, 1915.

1,160,041.

Patented Nov. 9, 1915.

*Fig. 1.*



*Fig. 2.*



*Fig. 3.*



*Fig. 4.*



Witnesses.—

Charles H. York  
Willard Burrows

Inventor.—

Charles E. Carpenter  
by his Attorneys.  
Howden & Howden

# UNITED STATES PATENT OFFICE.

CHARLES E. CARPENTER, OF PHILADELPHIA, PENNSYLVANIA.  
COMPOSITE LEATHER BELT.

Specification of Letters Patent.

Patented Nov. 9, 1915.

1,160,041.

Application filed February 5, 1915. Serial No. 6,307.

To all whom it may concern:

Be it known that I, CHARLES E. CARPENTER, a citizen of the United States, residing in Philadelphia, Pennsylvania, have invented certain Improvements in Composite Leather Belts, of which the following is a specification.

My invention relates to composite or built-up belts of leather; and the object of 10 my invention is to provide an improved belt of this character in which I combine leather prepared by the well known vegetable tannage with leather made by mineral tannage or, as it is more familiarly known, 15 "chrome tannage."

My improved belt is made of a plurality of plies of leather, two or more as the case may be, one of which plies is of vegetable tanned leather.

20 My improved composite belt made of vegetable and mineral tanned leather possesses a number of peculiar advantages. In the first place, while leather made by mineral tannage is tougher, stronger and more 25 supple and yielding than leather made by vegetable tannage, it is also susceptible of greater stretch hence, except in the case of very heavy hides, a belt made wholly of mineral tanned leather is liable to stretch 30 excessively, and to narrow to such an extent as to substantially destroy its value. Vegetable tanned leather, on the other hand, is much stiffer, has relatively little stretch with no tendency to narrow in use, but lacks 35 suppleness and is liable to crack on the grain side when passing around small pulleys. By combining these respective leathers in the making of my improved composite belt, I take advantage of the qualities which 40 make each of them peculiarly valuable and produce a belt that partakes of or possesses the virtues of both leathers while avoiding their deficiencies.

In the use of leather belts there are times 45 and conditions when a tight hold or grip upon the pulley, without slip, is absolutely essential to the proper operation of the belt. Under other conditions it is of material advantage for a certain amount of slip 50 to occur; there being instances where it is absolutely necessary that the belt should slip at intervals in order that the proper operation of the structure with which it is used may be effected. In using my two-ply composite belt therefore, the mineral tanned

side may be in engagement with the pulley where no slip is required or desired, and the vegetable tanned leather may be in engagement with the pulley when conditions require or it is desired that slip shall take 60 place between the belt and the pulley.

Further, by the use of a belt with a layer of mineral tanned leather I am able to secure a better adherence to the pulley and effect a considerably greater pull per square 65 inch of contact with the pulley than under the best conditions with belts made wholly of vegetable tanned leather. Should slip occur when the mineral tanned leather side of the belt is in contact with the pulley, 70 there will be less danger of burning, since the mineral tanned leather is capable of 75 withstanding a temperature considerably higher than leather tanned by any of the vegetable processes.

These and other features of my invention are more fully described hereinafter, reference being had to the accompanying drawings, in which:

Figure 1, is a sectional view of an ordinary belt made wholly of vegetable tanned leather; Fig. 2, is a similar sectional view of a two-ply composite belt made in accordance with my invention; Fig. 3, is a sectional view of one form of three-ply composite belt made in accordance with my invention; 85 Fig. 4, is a sectional view of another form of three-ply composite belt made in accordance with my invention.

In Fig. 1, which shows a section of an ordinary composite leather belt as heretofore made, the grain sides of two layers 1, 1, of vegetable tanned leather form the outer or external surfaces of the belt, while the flesh sides or surfaces are secured together by a suitable cement that will insure proper engagement and contact throughout their length.

In Fig. 2, which shows a sectional view of my improved composite belt, 1 represents a layer of leather made in the ordinary manner with a vegetable tannage, such for instance as that employed in making the belt shown in Fig. 1, and 2 is a section of mineral tanned leather; the two sections of vegetable and mineral tanned leather being placed with their flesh sides in contact and secured together by cement of proper character or other suitable means that will insure permanent connection of said leather 110

sections for the purpose desired. The ply of mineral tanned leather may be thinner than the ply of vegetable tanned leather.

In preparing a three-ply belt, such as shown in Fig. 3, I prefer to employ a central part or core 1 of vegetable tanned leather, which is faced on both sides with plies 2 of mineral tanned leather. By this construction I am enabled to produce a belt having a high degree of suppleness, and further, one that is not susceptible of stretch; at the same time a belt so made will not crack or split, even when employed with pulleys of small size. In some instances I may employ two layers of vegetable tanned leather 1, 1, with a single layer of mineral tanned leather 2 at one side as clearly illustrated in Fig. 4. In my improved belt such as I have described, the plies of leather being of different tannage are liable to differences in elongation when subjected to severe tensile strains. Unless the cementitious body holding the plies together is elastic, there is danger of such plies separating under the strain, but by the employment of an elastic, water-proof cement, all danger of separation is avoided and a belt so constructed possesses the greatest possible efficiency.

While there are perhaps many cements available for securing together plies of leather, I have found that an elastic, water-proof cement is the best material that can be employed for securing together the plies of leather employed in making my improved composite belt. There may be many forms of water-proof cements available for the purpose, but I prefer to use a cement composed of gun cotton dissolved in acetone, or any cement of the celluloid group. When employing a cement of gun cotton and acetone I prefer a saturated solution of substantially sixteen (16) ounces of gun cotton to one (1) gallon of acetone.

In employing the cementitious body for securing together the respective plies of leather, I prefer to preliminarily size or coat the surfaces to be united with a thin body of the cement, which surfaces are then allowed to set or become substantially dry. Then the main coating of cement to effect the union of the plies is applied to these preliminarily coated surfaces, and after the plies have been placed together they may be subjected to pressure suitably applied until the cementitious body has acquired the desired set and effected permanent union of the respective leathers.

A composite belt which includes a ply of mineral tanned leather and a ply of vegetable tanned leather has many advantages; that is to say, the vegetable tanned leather corrects the defects of the mineral tanned leather, and the mineral tanned leather corrects the defects of the vegetable tanned leather. Mineral tanned leather when used

by itself has a greater tendency to stretch than vegetable tanned leather since it does not have sufficient body or firmness to enable it to hold its width under tension. Vegetable tanned leather, however, having firmness and great body enables the mineral tanned leather to hold its full width and avoid stretch when cemented or otherwise permanently secured thereto.

The mineral tanned skin is materially softer than the vegetable tanned skin, and is particularly desirable for contact with the pulley when slippage is to be avoided. While the mineral tanned leather is also much tougher than the vegetable tanned leather, any tendency of the mineral tanned leather to stretch, due to its softness, would be resisted by the vegetable tanned leather to which it is firmly secured, with the result of attaining all of the advantages possessed by a belt made of the best vegetable tanned leather, while avoiding all of the disadvantages of the same.

By reason of the supple character of the mineral tanned leather, it will have a tendency to cling more tightly to the pulley, and there will be very much less likelihood of any slip occurring. In case of slip, however, the danger of burning would be much less since the mineral tanned leather will stand a much higher temperature than vegetable tanned leather; probably as much as a difference of 100° F.

Such a belt while having greater strength than a belt of the same number of plies made of vegetable tanned leather, will be considerably lighter in weight and thereby effect economy in the load; that is to say, there will be less weight of belt to be pulled.

A great disadvantage in connection with the use of vegetable tanned leather belts when made of a plurality of plies is because the grain side of the belt is so apt to crack when the belt is bent, especially when passing around a small pulley. This is entirely avoided by the use of a mineral tanned skin as one of the plies or layers.

My improved composite belt will be far more supple than any double or triple composite vegetable tanned leather belt heretofore made, and hence will give better service when used in connection with small pulleys, particularly those of electric generators, and others driven at high speeds. Finally, its economy in weight with a gain in strength and efficiency of action will materially enhance its value without increasing the cost.

To sum up, my improved composite belt, made of independent layers or plies of vegetable tanned leather and mineral tanned leather cemented together, is capable of wider use than the ordinary composite belts; it is stronger; it will not crack in making short turns, passing over small pulleys and

the like; it will not slip when the face of mineral tanned leather is in contact with the pulley but can slip when the vegetable tanned leather face is in contact with the 5 pulley; and finally, while having a greater degree of suppleness, it will not lose its width in use, nor stretch.

A particular advantage in belts of the character described, when using a cement of 10 the celluloid group to secure the sections of the belt together, is that the two plies of belts being of different tannage are at times apt to be of varied elongation when subject to severe tensile strength, and where the ordinary cement is used the cement not being so elastic is apt to part under the strain, while with the cement such as is herein described, namely, a cement of the celluloid group, there is no such effect.

20 I claim:

1. A composite belt made up of a plurality of sections of mineral tanned leather and vegetable tanned leather, permanently secured together by a cement of the celluloid group.

2. A composite belt made up of a plurality of sections or plies of leather permanently secured together by a cement of the celluloid group.

30 3. A composite belt made up of a section of vegetable tanned leather, and a section of mineral tanned leather, permanently secured together by a cement of the celluloid group.

35 4. A composite belt made up of a plu-

rality of sections or plies of leather permanently secured together by a cement consisting of gun cotton in solution with acetone.

5. A composite belt made up of a section of vegetable tanned leather, and a section 40 of mineral tanned leather, permanently secured together by a cement consisting of gun cotton in solution with acetone.

6. A composite belt made up of a section of vegetable tanned leather, and a section of 45 mineral tanned leather having the flesh sides or surfaces of the same permanently cemented together by a cement of the celluloid group.

7. A composite belt made up of a section 50 of vegetable tanned leather, and a section of mineral tanned leather, said sections having their grain sides outermost with their flesh sides permanently secured together by a cement of the celluloid group.

55 8. A composite belt made up of a section of vegetable tanned leather, and a section of mineral tanned leather, said sections having their grain sides outermost with their flesh sides permanently secured together by a cement 60 consisting of gun cotton in solution with acetone.

In testimony whereof, I have signed my name to this specification, in the presence of two subscribing witnesses.

CHARLES E. CARPENTER.

Witnesses:

GEORGE H. MORGAN,  
CHARLES P. STOCKE.

Copies of this patent may be obtained for five cents each, by addressing the "Commissioner of Patents, Washington, D. C."